

Sept. 27, 1949.

S. SMITH

**2,482,945**

## METHOD OF FLAME HARDENING

Filed Sept. 25, 1946

2 Sheets-Sheet 1



FIG. 2



FIG. I

INVENTOR  
*STEPHEN SMITH*

BY  
Pennington, Edwards, Morton & Barrons  
ATTORNEYS

Sept. 27, 1949.

S. SMITH

2,482,945

METHOD OF FLAME HARDENING

Filed Sept. 25, 1946

2 Sheets-Sheet 2



FIG. 3

INVENTOR  
STEPHEN SMITH

BY

*Perkins, Edwards & Parke, Attorneys*

## UNITED STATES PATENT OFFICE

2,482,945

## METHOD OF FLAME HARDENING

Stephen Smith, Jersey City, N. J., assignor to Air Reduction Company, Incorporated, New York, N. Y., a corporation of New York

Application September 25, 1946, Serial No. 699,285

1 Claim. (Cl. 148—21.56)

1

This invention relates to the hardening of cylindrical surfaces of cast iron, steel and the like, and particularly to an improved method of effecting such hardening.

It has been proposed heretofore to harden the surface of a cylindrical body, especially an internal surface such as the inside of a pump liner, by subjecting the surface to flame heating, in a relatively narrow circumferential zone, to a temperature above the critical range for the metal, and progressively heating the adjoining metal further and further beyond the starting zone to a temperature above the critical range, and quenching the heated metal by the application of a cooling medium, such as water, the quench being advanced along the surface of the metal progressively at some distance behind the heating flames. The products of combustion from the heating flames pass upward along the surface of the work piece ahead of the flame and cause a preheating of the metal. Conduction of heat from the highly heated regions to the cooler metal ahead of the flame causes additional preheating.

The area toward the end of the work piece, that is the part last heated and quenched, is subjected to this preheating action for the longest time; and as the heating flames approach the end of the work piece there is less and less metal ahead of the flames for absorbing the heat that travels through the metal by conduction. These two factors cause the metal toward the end of the work piece to be more highly heated than the metal below it, if the heating flames progress at a substantially uniform speed. With such uneven heating, the hardening of the work piece is not uniform throughout its length.

Obviously attempts to progressively increase the speed of travel of the heating device complicate the apparatus used and introduce other difficulties such as the determination of the desirable increment of speed for each thickness and length of work piece to be treated. Successful hardening cannot be assured in an operation which introduces factors not readily determinable and not easily fulfilled.

It is the object of the present invention to provide an improved method of hardening surfaces of cast iron, steel and the like which avoid the disadvantages mentioned and permit an economical and practicable application of sufficient heat to quickly bring a narrow circumferential zone of the surface to a temperature above the critical range for the metal and to advance the heat progressively followed by a quench.

2

Other objects and advantages of the invention will be apparent as it is better understood by reference to the following specification and the accompanying drawing, in which

5 Fig. 1 is a sectional view showing a suitable heating device for the practice of the invention disposed in a cylindrical work piece in operative position to permit application of the method for hardening the surface;

10 Fig. 2 is a fragmentary sectional view, taken on the line 2—2 of Fig. 1; and

Fig. 3 is an elevation of a driving mechanism adapted to permit manipulation of the device to secure the desired result.

15 In describing the invention in more detail, reference is made particularly to the treatment of internal cylindrical surfaces. The invention may, however, be applied with similar results to external surfaces by suitable modification of the

20 apparatus employed, including, for example, an annular torch head in place of the torch head as hereinafter described. The invention is intended primarily for vertically disposed work pieces.

25 The invention involves the application of a plurality of heating flames to a narrow circumferential zone of the surface to be treated and the advancing of the flames progressively, followed closely by jets of a quenching medium such as water or cold gas directed against the heated metal.

30 Instead of having the hot gases of combustion and envelope gases preheat the surface before application of the heating flames thereto, these gases are diluted and cooled to a relatively low temperature by a blast of cold air or other cooling gas which is directed against the surface to be treated above the heating zone. Preheating of the surface by the combustion gases is prevented, and heat conducted by the metal from the heating zone into adjoining zones is dissipated by the impinging stream of cold gas. Thus, as each portion of the surface comes under the heating flames, the metal is at a relatively low and substantially uniform temperature and is rapidly heated to the critical temperature, and thereafter is immediately quenched.

35 This operation has four immediate and desirable effects. The blast of cold gas cools the metal by direct contact and thus reduces conduction of heat in the metal upward from the heating zone. It causes the envelope gases to burn closer to the region of primary heating and thereby concentrates the heat nearer the region where it is wanted. The cold gas also dilutes the products of combustion, sufficient volume of

the cold gas being used to cool the products of combustion to the point where their heating effect on the metal above the heating zone is no longer objectionable. The metal ahead of the heating zone is kept at a substantially uniform temperature so that a constant depth of heating and surface temperature is obtained throughout the length of the work piece.

The procedure permits flame hardening to be carried on progressively and at constant speed, achieving a uniform depth of hardness from the bottom to the top of the surface under treatment. A further advantage is that the speed of movement of the heating device may be uniform throughout its path of travel, thereby avoiding the necessity for complicated mechanism necessary if the speed must be increased by successive increments because of excessive preheating of the surface.

The heating may be accomplished by combustion of any suitable combustible gas with oxygen or air, provided the necessary amount of concentrated heat can be applied as desired. Oxyacetylene flames are particularly adapted for the purpose, and these may be provided by employing a suitable torch head having means for supplying and mixing the gases and for discharging the mixture through a plurality of circumferentially disposed orifices. The torch head is also supplied with a quenching medium such as water or cold gas which is discharged through circumferentially disposed orifices below the heating orifices so as to impinge on the previously heated surface. Above the heating orifices are similar orifices supplied with a relatively large volume of a cooling gas such as air, jets of which impinge on the surface to be treated and mingle with the products of combustion and with the envelope gases, thus maintaining the low temperature of the surface by preventing preheating thereof and by withdrawing heat transferred through the metal from the heating zone. The volume of cooling gas should be such as to reduce very materially the temperature of the combustion and envelope gases, though the exact temperature is not critical.

The torch head may be mounted in any suitable manner to permit movement thereof at a uniform rate upwardly as the hardening operation progresses. Thus water, if used as a quenching agent, will run downwardly without interfering with the heating.

Referring to Fig. 1 of the drawing, 2 indicates a fixture having a bore 3 and a ledge 4 which is adapted to support a work piece 5 having a bore or cylindrical surface 6 which is to be hardened by the practice of the invention as described herein. A torch head 7 is supported on a tubular member 8 for vertical movement in the bore 6, preferably from the bottom upward, as herein-after described. The lower end of the tubular member 8 is secured to a block 9 which is threadedly connected to a tubular member 10 having a conical end 11 which fits snugly in a conical seat 12 of a block 13. A threaded nipple 14 is connected to the block 13 and a hose (not shown) may be secured to the nipple and connected with a source of oxygen which flows through the passage 15 in the tubular member 10. A threaded nipple 16, also secured to the block 13, is adapted to be connected by a hose (not shown) to a source of acetylene which flows through the passage 17 to a groove 18 and thence through inlets 19 into the mixing chamber 15 where it mixes

with the oxygen and provides the fuel to maintain the heating jets.

A tubular member 10' concentrically surrounds the member 10. One end of the member 10' seats on a ledge in the block 9 and the other end fits against the conical seat 12 of the block 13. The member 10' is secured to the block 13 by a nut 20 which holds the conical end of this member 10' firmly against the seat 12. A nut 21 surrounds the member 10' and engages the block 9, packing 22 being disposed behind the nut 21 to prevent leakage of quenching medium from passage 23 formed between the members 10 and 10'. This passage 23 communicates via a passage 24 (Fig. 2) with a nipple 25 which is adapted to be connected through a hose (not shown) with a source of quenching medium such as water or a cold gas.

Within the tubular member 8 are two concentric tubes 26 and 27, forming passages 28, 29 and 30. The end of the tube 27 terminates in a threaded nipple 31 which is adapted to be connected through a hose (shown dotted) with a source of air or other cooling gas under pressure. The latter is conducted through the tube 27 to a chamber 32 at the top of the torch head 7, and a plurality of orifices 33 distribute the cooling gas under pressure circumferentially about the torch head in a plurality of jets which impinge upon the cylindrical surface 6.

30 Directly below the chamber 32 is a chamber 34 which communicates with the passage 29 between the tubes 26 and 27. This passage in turn communicates with the mixing chamber 15, and thus the mixture of combustible and oxidizing gas is 35 delivered to the chamber 34 and distributed through a set of staggered orifices 35 disposed circumferentially about the torch head 7. When ignited, the gaseous mixture forms a plurality of 40 flame jets which impinge upon the cylindrical surface 6 to effect the desired heating thereof. Below the chamber 34 is a third chamber 36 communicating with the passage 28 formed between the tubular member 8 and the concentric tube 26, and this passage 28 communicates with a passage 45 37 that is connected by a passage 38 with the passage 23, thus affording a supply of quenching medium such as water to the chamber 36. The water is distributed through a plurality of circumferentially disposed orifices 40 in the torch 50 head 7 so that the quenching medium impinges upon the surface 6 below the flame jets. A deflecting shield 61 is removably attached to the fixture 2 by the supporting links 62 and rotatable dogs 63. The quench water falls on the deflecting shield 61 and is directed by a lip 64 to run off at the desired point.

To effect the vertical movement of the torch head 7, the block 9 may be mounted upon any suitable clamping device such as clamps 65 which are rigidly attached to a support 66 fixed to a base 67. This base 67 is supported by a piston rod 68 of a hydraulic cylinder 69 (Fig. 3). A fixed guide 70 maintains the torch head centered 65 in the work piece. Other apparatus capable of moving the torch vertically may be employed.

With the structure illustrated, the torch head 7 can be disposed below the lower edge of the surface 6, the combustible gas may be ignited to produce the flame jets and thereafter the torch head may be raised at a uniform speed through the work piece to be hardened. As the torch head 7 rises, each increment of the surface 6 is subjected successively to the cooling effect of 70 the cooling gases, is then heated rapidly to the

critical temperature and immediately thereafter is cooled by the cooling medium to reduce the temperature and effect the desired hardening of the surface.

The surface 6 above the level of the heating flames is continuously maintained at a relatively low and uniform temperature as the result of the large volume of cooling medium which continuously impinges on and flows upwardly over the surface. The hardening results are of uniform character.

Various changes may be made in the details of the operation and in the apparatus employed without departing from the invention or sacrificing the advantages thereof.

I claim:

The method of hardening cylindrical surfaces of a hardenable ferrous alloy which comprises positioning the cylindrical surface in a substantially vertical position, progressively moving jets of relatively cold gaseous medium axially and upwardly of the cylindrical surface and directing them onto the surface to be hardened to precool it to a substantially uniform temperature, pro-

gressively directing an annular row of heating flames against the precooled surface closely adjacent the portion of the surface against which the precooling gaseous medium is being directed, the intensity of the flames and the duration of their contact with the precooled surface being sufficient to bring the surface progressively to its critical temperature, and progressively directing jets of a quenching liquid onto the heated surface immediately beneath the zone of application of the heating flames.

STEPHEN SMITH.

#### REFERENCES CITED

- 15 The following references are of record in the file of this patent:

#### UNITED STATES PATENTS

| Number    | Name         | Date          |
|-----------|--------------|---------------|
| 2,065,627 | Taylor       | Dec. 29, 1936 |
| 2,279,564 | Emery et al. | Apr. 14, 1942 |
| 2,318,145 | Emery et al. | May 4, 1943   |
| 2,382,515 | Smith        | Aug. 14, 1945 |